

3,404,687

## CIGARETTE PAPER

James C. Rickards, Brevard, and William F. Owens, Jr., Pisgah Forest, N.C., assignors to Olin Mathieson Chemical Corporation, a corporation of Virginia  
No Drawing. Filed Dec. 23, 1966, Ser. No. 604,178  
1 Claim. (Cl. 131—15)

### ABSTRACT OF THE DISCLOSURE

This invention provides improved cigarette paper of high porosity to serve as wrapper for a cigarette tobacco column, which effects a significantly greater reduction of the vapor phase constituents of cigarette smoke than of the particulate constituents. Very high porosity is imparted to the paper by the provision of perforations having length and width dimensions between about 0.001 to 0.015 inch, the size and number being such as to impart to the paper an absolute Greiner porosity index value in the unprecedented low range of about 1 to 3. The perforations are symmetrically arranged with respect to the length and width of the paper, and preferably are arranged in the form of two or three longitudinal rows. The use of the improved cigarette paper of this invention results in cigarettes which yield smoke of reduced content both of vapor phase and particulate constituents, with selective reduction of the vapor phase constituents.

This invention relates to improved paper wrappers for cigarettes and like smoking devices and, more particularly, to improved cigarette paper which is provided with a plurality of perforations, preferably aligned in rows, said perforations being symmetrically spaced with respect to the length and width of the said paper. The arrangement of the perforations is such that when a cigarette tobacco column has been enclosed in a wrapper formed of the said paper, the perforations are distributed symmetrically with respect to the length and circumference of the cigarette.

The spaced perforations provided in the paper have length and width dimensions between about 0.001 to 0.015 inch, the size and number being so coordinated as to impart an absolute Greiner porosity index value, as hereinafter defined, within the range of about 1 to 3. Preferably, the perforations are provided in longitudinal alignment, desirably in two or three rows.

As will be apparent from the following detail description and illustrative embodiments, the provision of cigarette paper wrappers as above defined in accordance with this invention surprisingly enables the attainment of significant advantages.

Many prior proposals have been made for the use of porous cigarette wrapper paper, particularly of paper which has been rendered porous by a perforating treatment, the purpose being to attenuate and cool the smoke. Typical examples were discussed and referred to in the article "The Design of Low Yield Cigarettes" by Schur and Rickards, *Tobacco Science*, vol. 4, pp. 69-77 (1960)

and in U.S. Patent 3,046,994 issued to Milton O. Schur on July 31, 1962.

On the basis of comparative smoking tests of cigarettes provided with wrappers having a Greiner porosity index of about 10 (absolute value of about 6) attained by a variety of methods, the conclusion stated in the latter disclosure was that essentially the same reduction in particulate content and in contents of gaseous components were found (U.S. 3,046,994 col. 6, lines 48-68).

It has now been discovered that a selective reduction of vapor phase constituents in cigarette smoke can be effected by the provision of paper wrappers having much higher porosities, in the range of absolute Greiner porosity index values of about 1 to 3, wherein the porosity is imparted to the wrapper through the provision of symmetrically distributed spaced perforations having length and width dimensions of 0.001 to 0.015 inch. Preferably, such perforations are provided as two or three longitudinal rows, both the perforations and the rows being equally spaced from the adjacent ones in the assembled cigarette. The use of such paper wrappers provides a substantially greater reduction of vapor phase constituents of the cigarette smoke than of the particulate matter, the ratio of percentage reductions generally being about 1.5, and within the range of 1.1 to 2. In other words, cigarette papers perforated in accordance with this invention display a selective reduction of vapor phase constituents of cigarette smoke.

Such selectivity has now been shown to occur uniquely within a range of porosities corresponding to the relatively narrow range of absolute Greiner porosity index values of about 1 to 3, representing porosities much greater than any heretofore proposed as suitable for cigarette wrappers. With respect to such porous wrappers of the prior art, displaying a maximum porosity corresponding to a Greiner porosity index value of about 10 (absolute value of 6) or some lower porosity corresponding to a higher index value, the general belief, as supported by the available data, has been that such wrappers effected a reduction in concentration of all smoke constituents equally at a given porosity index value. For such wrappers, the selectivity ratio is 1, this ratio being defined as the quotient of the percentage reduction of vapor phase constituents of the smoke divided by the percentage reduction of the particulate constituents.

The accomplishment of the selective reduction of vapor phase constituents of cigarette smoke in accordance with this invention requires the provision of a porous cigarette paper characterized by an absolute Greiner porosity index value of about 1 to 3, with said porosity being imparted by symmetrically arranged macroscopic perforations. Such selective reduction is not attained with the use of paper characterized by the stated range of porosity index values, wherein the porosity is imparted by other means, for example by the provision of sufficient microscopic or submicroscopic openings.

The above conclusions were based on the results of comparative experiments of smoking tests as summarized in Tables I and II, characterizing, respectively, the advantageous performance in accordance with this invention as contrasted with the confirmation of what might have been expected from the prior art.

TABLE I

| Cigarette paper                     | Abs. Greiner porosity (sec./50 ml.) | Particulate phase |                   | Vapor Phase, Av. Percent Reduction | Selectivity ratio |
|-------------------------------------|-------------------------------------|-------------------|-------------------|------------------------------------|-------------------|
|                                     |                                     | Yield (mg./cig.)  | Percent Reduction |                                    |                   |
| Control                             | 19.1                                | 32.1              |                   |                                    |                   |
| 1.....Macroscopic perforations..... | 0.5                                 | 13.6              | 57.7              | 64.7                               | 1.12              |
| 2.....do.....                       | 1.0                                 | 21.6              | 32.7              | 44.6                               | 1.37              |
| 3.....do.....                       | 1.7                                 | 23.6              | 26.5              | 39.3                               | 1.48              |
| 4.....do.....                       | 2.0                                 | 24.5              | 23.7              | 34.5                               | 1.46              |
| 5.....do.....                       | 3.1                                 | 25.5              | 20.5              | 29.5                               | 1.44              |
| 6.....do.....                       | 4.0                                 | 26.4              | 17.7              | 21.0                               | 1.18              |

TABLE II

| Cigarette paper                      | Abs. Greiner porosity (sec./50 ml.) | Particulate phase |                   | Vapor Phase, Av. Percent Reduction | Selectivity ratio |
|--------------------------------------|-------------------------------------|-------------------|-------------------|------------------------------------|-------------------|
|                                      |                                     | Yield (mg./cig.)  | Percent Reduction |                                    |                   |
| Control                              | 19.1                                | 32.1              |                   |                                    |                   |
| a..... Inherently porous.....        | 1.0                                 | 16.4              | 48.8              | 40.6                               | 0.83              |
| b..... do.....                       | 1.5                                 | 17.8              | 44.6              | 39.8                               | 0.90              |
| c..... do.....                       | 2.0                                 | 17.8              | 44.6              | 37.7                               | 0.85              |
| d..... do.....                       | 3.1                                 | 21.4              | 33.3              | 34.7                               | 1.05              |
| e..... do.....                       | 4.1                                 | 25.2              | 21.5              | 18.5                               | 0.86              |
| f..... Microscopic perforations..... | 0.8                                 | 14.7              | 54.2              | 52.9                               | 0.98              |
| g..... do.....                       | 1.5                                 | 20.4              | 36.3              | 31.6                               | 0.87              |
| h..... do.....                       | 2.0                                 | 21.3              | 33.6              | 32.3                               | 0.96              |
| i..... do.....                       | 2.8                                 | 22.4              | 30.2              | 24.3                               | 0.80              |
| j..... do.....                       | 3.8                                 | 22.7              | 29.2              | 15.4                               | 0.53              |

The above results show that the greatest selective reduction of vapor phase constituents was effected with the use of macroscopically perforated paper listed in Table I, in the range of 1 to 3 seconds absolute Greiner porosity index. No such selectivity was shown in the same range of porosities with the papers listed in Table II.

The test cigarettes of these two tables were prepared by wrapping the tobacco column of the same popular commercial brand of cigarette in wrappers of the same paper, which differed only as indicated with respect to the porosity value and the manner of imparting porosity.

In Examples 1 to 6 of Table I, the macroscopic perforations were produced by means of apparatus as shown in U.S. Patent 2,699,208 issued Jan. 11, 1955, to Milton O. Schur to provide two longitudinal rows of perforations, symmetrically spaced apart so that in the wrapped cigarette the rows of perforations are equally spaced from each other. In Examples 1 and 2, there were 30 perforations per inch along each row, produced by rectangular perforating teeth which were initially 0.010 inch in length and 0.001 inch in width. The lower porosity of Example 2 could be produced by the use of lower perforating pressures or of somewhat worn perforating rolls. In Examples 3 and 4, there were 16 perforations per inch along each row, produced by perforating teeth which were initially 0.005 inch by 0.005 inch. In Examples 5 and 6, there were 8 perforations per inch along each row, produced by rectangular perforating teeth which were initially 0.010 inch in length and 0.0025 inch in width. The resulting perforations may be characterized as macroscopic in that they are visible without magnification at normal reading distances.

In contrast, the papers listed in Table II were rendered porous by the production of microscopic openings, through control of the papermaking process, particularly with respect to the extent of beating, in samples *a* to *e* and mechanically in samples *f* to *j*, which were prepared which were prepared as described in U.S. Patent 3,179,025, issued Apr. 20, 1965, to Milton O. Schur. For example, sample *h*, displaying an absolute Greiner porosity index value of 2.0, was found to contain approximately 75 perforations per square centimeter averaging about 60 microns in diameter.

The porosity index values were measured with the use of a Greiner porosity tester, an instrument long used in the paper industry. The measurement is of the time in seconds for 50 ml. of air to be drawn through a test area of paper one inch in diameter under the influence of a varying suction head corresponding to a column of water averaging about 4½ inches in height. The readings have been corrected to absolute values by deducting the time, close to 4 seconds, required for a blank determination, without any paper sample in the instrument. For increased accuracy, the time measurements were carried out automatically by the use of a light absorbing solution and a photo-electric circuit in the apparatus. It will be seen that the time of flow increases with decreasing porosity of the paper sample, and thus, the lower the value of the measured index the more porous is the paper. In testing, care was taken in placing the sample so that the perforations

if any were symmetrically arranged with respect to the center of the orifice.

The smoking tests reported herein were carried out in conventional manner, a 35 ml. puff being taken over a two second interval once per minute. In every case, 47 mm. of each cigarette was smoked, using cigarettes which had been conditioned for at least 48 hours at 72° F. and relative humidity of 63%. The cigarettes were selected by weight to be within  $\pm 2\%$  of the average weight of the group under test.

Particulate matter was removed from the smoke by means of a Cambridge Absolute Filter and weighed.

The quantitative determination of vapor phase constituents was carried out by gas chromatography, generally as described by Irby and Harlow in *Tobacco Science* vol. 3, 52-56 (1959). The average reduction corresponds to the average of the reductions determined with respect to the eleven constituents listed in Table III.

The smoke analysis results in Table III were obtained on cigarettes prepared by wrapping the tobacco column of a popular commercial brand of cigarettes (not the same as used in the preceding tables) in a standard cigarette paper. Testing was carried out both with cigarettes having unperforated wrappers and having wrappers perforated as in Example 4 above (two lines of  $0.005 \times 0.005$  inch perforations, 16 per inch).

TABLE III

| Smoke Constituent         | Unperforated (mg./cig.) | Perforated (mg./cig.) | Percent reduction | Selectivity ratio |
|---------------------------|-------------------------|-----------------------|-------------------|-------------------|
| Particulates.....         | 27.65                   | 21.20                 | 23.3              | .....             |
| Vapor phase constituents: |                         |                       |                   |                   |
| Isoprene.....             | 0.75                    | 0.40                  | 46.6              | 2.00              |
| Acetaldehyde.....         | 1.02                    | 0.58                  | 43.1              | 1.85              |
| Acetone.....              | 0.48                    | 0.33                  | 31.2              | 1.34              |
| Methanol.....             | 0.24                    | 0.20                  | 16.7              | 0.72              |
| Methyl furan.....         | 0.051                   | 0.038                 | 25.5              | 1.10              |
| Methyl ethyl ketone.....  | 0.119                   | 0.084                 | 20.4              | 1.26              |
| Furan.....                | 0.038                   | 0.025                 | 34.2              | 1.47              |
| Propionaldehyde.....      | 0.076                   | 0.043                 | 43.4              | 1.87              |
| Acrolein.....             | 0.122                   | 0.065                 | 46.7              | 2.01              |
| Methyl acetate.....       | 0.016                   | 0.009                 | 43.8              | 1.88              |
| Isobutyraldehyde.....     | 0.032                   | 0.021                 | 34.4              | 1.47              |
| Average.....              |                         |                       | 35.9              | 1.54              |

The average selectivity ratio of 1.54, confirms the selective reduction of vapor phase constituents in accordance with the invention. The non-selectivity found with respect to methanol occurs occasionally with respect to one or several constituents and is believed to be characteristic of the particular tobacco blend.

The general applicability to a variety of tobacco blends is illustrated in Table IV, wherein the analytical results were obtained with 12 different commercial brands of cigarettes produced by various manufacturers. In each case, the cigarette tobacco column was wrapped in a paper wrapper identical to the others, excepting that the controls were unperforated and the others were perforated. In the perforated wrappers, the openings were provided as in Example 4.

TABLE IV

| Brand | Particulate phase,<br>Percent reduction | Vapor phase,<br>Percent reduction | Selectivity<br>ratio |
|-------|-----------------------------------------|-----------------------------------|----------------------|
| A     | 23.2                                    | 35.9                              | 1.54                 |
| B     | 35.8                                    | 39.3                              | 1.10                 |
| C     | 27.3                                    | 40.9                              | 1.50                 |
| D     | 19.0                                    | 36.6                              | 1.93                 |
| E     | 21.4                                    | 42.8                              | 2.00                 |
| F     | 25.9                                    | 35.9                              | 1.38                 |
| G     | 23.3                                    | 34.9                              | 1.50                 |
| H     | 15.8                                    | 24.0                              | 1.52                 |
| I     | 41.3                                    | 49.1                              | 1.20                 |
| J     | 32.4                                    | 34.6                              | 1.07                 |
| K     | 17.0                                    | 36.4                              | 2.14                 |
| L     | 17.7                                    | 28.9                              | 1.63                 |

Brands A through H were 70 mm. unfiltered cigarettes, brands I through K were 85 mm. unfiltered cigarettes and brand L was an 85 mm. cigarette provided with a filter of cellulose acetate filaments.

Table V, listing smoking test results of a domestic blend of cigarette tobaccos, likewise establishes a selective reduction with respect to the content in the smoke of nitrogen oxides, expressed as nitrogen dioxide. Comparative tests were made as outlined above of the domestic blend tobacco wrapped in two different types of cigarette paper.

The selective reduction in vapor phase constituents of tobacco smoke, thus accomplished in accordance with this invention, advantageously improves the taste and flavor. Some of these constituents are known to be acrid, irritating or a least unpleasant and the above-described significant lowering in the concentration thereof is beneficial.

The attainment of such selective reduction by using a wrapper of macroporous paper, in contrast to the absence of any selective decrease when a microporous wrapper is used was a surprising as well as advantageous result. Although a verified explanation is not available, it seems probable that the effectiveness of the macroporous paper wrappers of this invention is based on the entrance of lateral air jets into the cigarette when it is puffed which impinge upon the burning zone with sufficient velocity to effect a more complete combustion. Such jets have a far higher velocity than the many streams of air entering through a much greater number of tiny pores in a microporous wrapper.

In support of the obtainment of more complete combustion at or near the burning zone, it has been determined that generally, lower carbon monoxide content of the smoke results with the use of macroporous rather than microporous paper wrappers, all characterized by

TABLE V

| Cigarette paper       | Particulate phase   |                      | Nitrogen dioxide    |                      | Selectivity<br>ratio |
|-----------------------|---------------------|----------------------|---------------------|----------------------|----------------------|
|                       | Yield<br>(mg./cig.) | Percent<br>reduction | Yield<br>(mg./cig.) | Percent<br>reduction |                      |
| Paper A, unperforated | 35.6                |                      | 148.0               |                      |                      |
| Paper A, perforated   | 29.0                | 18.4                 | 109.0               | 26.2                 | 1.42                 |
| Paper B, unperforated | 38.3                |                      | 123.0               |                      |                      |
| Paper B, perforated   | 28.8                | 24.8                 | 70.2                | 43.0                 | 1.73                 |

The perforated papers were provided with two longitudinal lines of 0.005 by 0.005 inch openings at a density of sixteen per inch. The determinations of nitrogen oxides as nitrogen dioxide were made essentially according to the Salzman procedure, Analytical Chemistry vol. 16, 40 272-274 (1947).

In contrast with the above-described selective reduction of nitrogen oxides from the smoke with the use of macroporous cigarette paper as wrapper, comparative tests with microporous paper, having an absolute Greiner porosity index within the range of 1 to 3 imparted inherently by the paper making process or mechanically, showed the absence of such selective reduction.

A similar contrast in smoking test results was established with respect to nitrogenous compounds in the vapor phase of the smoke, as set forth in Table VI.

an absolute Greiner porosity index in the range of 1 to 3. Furthermore, this is paralleled by a greater percentage reduction in the carbon monoxide content than with respect to carbon dioxide.

It has further been indicated that the macroscopic perforations must be symmetrically arranged, in addition to being sufficient in size and number to impart a porosity in the effective critical range. Departures from symmetry in the arrangement of the perforations tends to decrease significantly the selectivity effect.

It should be emphasized that the selectivity effect is attained within the critical range of paper porosities corresponding to absolute Greiner porosity index values of about 1 to 3, a value of about 2 being preferred. At Greiner porosity index values less than 1 and substantially greater than 3, the selectivity effect decreases or

TABLE VI

| Cigarette paper        | Abs. Greiner<br>porosity<br>(sec./50 ml.) | Particulate<br>phase,<br>percent<br>reduction | Vapor phase<br>N. cmpds.,<br>percent<br>reduction | Selectivity<br>ratio |
|------------------------|-------------------------------------------|-----------------------------------------------|---------------------------------------------------|----------------------|
| Control, unperforated  | 19.1                                      |                                               |                                                   |                      |
| 7. Macroporous         | 1.0                                       | 36.8                                          | 49                                                | 1.33                 |
| 8. do                  | 1.6                                       | 29.9                                          | 38                                                | 1.27                 |
| 9. do                  | 2.0                                       | 27.1                                          | 34                                                | 1.26                 |
| 10. do                 | 3.0                                       | 21.8                                          | 30                                                | 1.38                 |
| 11. do                 | 4.0                                       | 17.5                                          | 28                                                | 1.60                 |
| Microporous            | 0.8                                       | 54.2                                          | 53                                                | 0.98                 |
| do                     | 1.6                                       | 36.5                                          | 36                                                | 1.00                 |
| do                     | 1.8                                       | 33.6                                          | 28                                                | 0.83                 |
| do                     | 3.0                                       | 30.2                                          | 22                                                | 0.73                 |
| do                     | 4.0                                       | 29.2                                          | 27                                                | 0.91                 |
| Inherently microporous | 1.0                                       | 48.9                                          | 38                                                | 0.78                 |
| do                     | 1.6                                       | 44.6                                          | 43                                                | 0.98                 |
| do                     | 2.0                                       | 44.6                                          | 29                                                | 0.64                 |
| do                     | 3.1                                       | 33.3                                          | 35                                                | 1.05                 |
| do                     | 4.0                                       | 21.5                                          | 22                                                | 1.02                 |

Examples 7 to 11 above were perforated as previously described Examples 2 to 6 (Table I), respectively. The total nitrogenous compounds in the vapor phase were determined by converting them to nitrates through oxidation with potassium permanganate, the amount of nitrate being then measured by a known procedure.

70 vanishes. Also, at values less than 0.5, difficulties arise in easily lighting the cigarette.

The macroscopic perforations should have a length and width dimensions within the range of 0.001 to 0.015 inch. Larger openings are undesirable as tending to weaken the paper or tending to detract from the appearance,

while smaller openings decrease or eliminate the selectivity effect. The shape of the perforations may be varied as desired, provided that the area of the openings is within the specified macroscopic range. Thus, circular, elliptical, crescent, or partially circular, as well as triangular, rectangular or other polygonal shapes are suitable. When the perforating method and apparatus issued is as shown in U.S. Patent 2,699,208, the perforations should be square or rectangular. However, other methods of perforation may be employed, for example as set forth in U.S. Patents 3,074,303 or 3,021,732. The provision of two or three lines of regularly spaced perforations is preferred as an effective product can thus be made readily and efficiently at high production rates.

The selective reduction of vapor phase constituents in accordance with this invention may be applied advantageously to any type of cigarette, including cigarettes provided with any of the available types of filters. Particular advantages may be derived in filter cigarettes combining macroporous paper wrappers as defined herein with a specialized filter tip adapted to remove certain components from the smoke or to supply flavoring ingredients to the smoke.

What is claimed is:

1. A cigarette paper adapted to serve as wrapper for 25 a tobacco column,

5

10

15

20

said paper being provided with a plurality of macroscopic perforations aligned longitudinally in lines containing about 8 to 30 perforations per inch arranged symmetrically about the center of said paper, said perforations having length and width dimensions between .001 and .015 inch and imparting to said paper an absolute Greiner porosity index of about 1 to 3,

whereby smoke drawn from a cigarette tobacco column wrapped with said paper is attenuated by a plurality of substantially symmetrically disposed jets of air directed inwardly through said column, thereby effecting a significant reduction both of vapor phase and particulate constituents of said smoke with selective reduction of said vapor phase constituents.

#### References Cited

##### UNITED STATES PATENTS

3,046,994 7/1962 Schur ----- 131—15

##### FOREIGN PATENTS

998,557 9/1951 France.

594,627 6/1959 Italy.

683,748 4/1964 Canada.

MELVIN D. REIN, *Primary Examiner.*

**PATENT OFFICE**

**Washington, D.C. 20231**

**UNITED STATES PATENT OFFICE**  
**CERTIFICATE OF CORRECTION**

Patent No. 3,404,687

October 8, 1968

James C. Rickards et al.

It is certified that error appears in the above identified patent and that said Letters Patent are hereby corrected as shown below:

Column 3, line 53, cancel "which were prepared". Column 4, lines 39 and 40, "perforated" should read -- perforated --. Columns 5 and 6, TABLE V, sub-heading of the fourth column, "Yield (mg./cig.)" should read -- Yield ( $\mu$ g./cig.) --. Column 6 line 5, "a" should read -- at --; line 72, cancel "a".

Signed and sealed this 3rd day of March 1970.

(SEAL)

Attest:

Edward M. Fletcher, Jr.

Attesting Officer

**WILLIAM E. SCHUYLER, JR.**

Commissioner of Patents

[Redacted]